

## UNITED STATES PATENT OFFICE.

FREDERICK M. BECKET, OF NIAGARA FALLS, NEW YORK, ASSIGNOR TO ELECTRO METALLURGICAL COMPANY, A CORPORATION OF WEST VIRGINIA.

## METHOD OF TREATING TIN-BEARING TUNGSTEN ORES.

No Drawing.

Application filed May 26, 1920. Serial No. 384,266.

*To all whom it may concern:*

Be it known that I, FREDERICK M. BECKET, a citizen of the United States, residing at Niagara Falls, in the county of Niagara and 5 State of New York, have invented certain new and useful Improvements in Methods of Treating Tin-Bearing Tungsten Ores, of which the following is a specification.

This invention is a method for the treatment of tin-bearing tungsten ores, and is 10 applicable for the preparation from such ores of tungsten metal or ferrotungsten commercially free from tin. The method is particularly applicable to the treatment of such 15 ores as Chinese wolframite, which often contains sufficient tin to render it practically worthless for many smelting operations, in the course of which tin is readily reduced. While such ores may vary considerably in 20 composition, the following may be regarded as typical:

|                       | Per cent. |
|-----------------------|-----------|
| WO <sub>3</sub> ----- | 69-71     |
| FeO-----              | 13-15     |
| MnO-----              | 9-11      |
| Sn-----               | 0.4-0.7   |

I have discovered that a commercially complete elimination of the tin may be secured by subjecting the properly ground 30 ore to a roasting operation within suitable temperature limits, and thereafter dissolving out the tungsten content by a suitable alkaline reagent, which is preferably caustic soda. The tungsten may be precipitated 35 from the resulting substantially tin-free sodium tungstate solution in the form of its calcium salt, which is then smelted in known manner for the preparation of metallic tungsten or its alloys with iron or other 40 metals.

Following is a specific example of my method, it being understood that the invention is not restricted to the specific operating conditions therein described:

45 A tin-bearing tungsten ore of the type mentioned above is rather finely ground, preferably to 40 mesh and finer; and the fine ore is then subjected to an oxidizing roast, preferably at a temperature range of about

460-720° C. Temperatures somewhat below 50 this range, say down to 300° C., may be employed with somewhat inferior results; but materially higher temperatures, say 900° C. or upward, render the tungsten content of the ore substantially insoluble and are therefore to be avoided. 55

The roasted ore is then treated with a hot caustic soda solution until substantially all of its tungsten content is dissolved. A 20% solution maintained just short of its boiling 60 temperature is satisfactory for this purpose. If necessary the residues from the first operation may be re-treated with fresh alkali.

The residue from this treatment should 65 contain substantially the whole of the tin content of the ore, together with practically all of its manganese and iron content, and may be discarded so far as the purposes of the present invention are concerned. The 70 tungsten content of the solution is precipitated, preferably as the calcium salt, and the latter is subjected to electric furnace reduction, preferably using silicon or other non-carbonaceous reducing agent in case a low- 75 carbon product is desired.

I claim:

1. Method of treating tin-bearing tungsten ores of the wolframite type, comprising roasting a suitably comminuted ore, and extracting the tungsten content thereof by an alkaline solvent, whereby a substantially tin-free solution is obtained. 80

2. Method of treating tin-bearing tungsten ores of the wolframite type, comprising 85 roasting a suitably comminuted ore, and extracting the tungsten content thereof by a caustic soda solution, whereby a substantially tin-free solution is obtained.

3. Method of treating tin-bearing tungsten ores of the wolframite type, comprising roasting a suitably comminuted ore at about 460°-720° C., and extracting the tungsten content thereof by an alkaline solvent, whereby a substantially tin-free solution is 95 obtained.

In testimony whereof I affix my signature.

FREDERICK M. BECKET.